# EUROPEAN PATENT APPLICATION

(11) **EP 4 782 125 A1**
(43) Date of publication of application: **29.07.2026**
(21) Application number: 24911875.3
(22) Date of filing: 17.09.2024
(51) Int. Cl.: B22D 11/124, B22D 11/20, B22D 11/22

(54) **CONTINUOUS CASTING METHOD FOR CAST SLAB**

(30) Priority: 26.12.2023 JP 2023218734
(71) Applicant: JFE Steel Corporation, Tokyo 100-0011 (JP)
(72) Inventor: KUMAGAI Atsushi, Tokyo 100-0011 (JP); KAMADA Kohei, Tokyo 100-0011 (JP); UENO Seigo, Tokyo 100-0011 (JP); MATSUMOTO Takuya, Tokyo 100-0011 (JP); OYAMA Satoshi, Tokyo 100-0011 (JP); KAMEDA Kiyohiro, Tokyo 100-0011 (JP); TANAKA Yoshiyuki, Tokyo 100-0011 (JP); IRIE Shuhei, Tokyo 100-0011 (JP); MORITA Shugo, Tokyo 100-0011 (JP); TOISHI Keigo, Tokyo 100-0011 (JP); ARAMAKI Norichika, Tokyo 100-0011 (JP)
(74) Representative: Haseltine Lake Kempner LLP
(86) International application number: PCT/JP2024/033020
(87) International publication number: WO 2025/141981

(57) **Abstract**

There is provided a slab continuous-casting method that is capable of improving productivity of a slab having a thickness larger than that of conventional slab and that is capable of ensuring surface quality of the slabs by suppressing surface cracks in the slabs.

In a slab continuous-casting method using a continuous casting machine that includes a mold 6, a vertical section 8 disposed downstream of the mold 6 in a moving direction of a slab 7 withdrawn from the mold 6, a bending section 10 disposed downstream of the vertical section 8 in the moving direction, and a horizontal section 11 disposed downstream of the bending section 10 in the moving direction, the surface temperature of the slab 7 at the exit side of the vertical section 8 is 700°C or higher and 1200°C or lower, and a first cooling density X calculated from an amount of cooling water in the bending section 10 is less than or equal to a second cooling density Y calculated from an amount of cooling water in the horizontal section 11.

## Description

### Technical Field

The present invention relates to a slab continuous-casting method.

### Background Art

Steel plates for boilers, low-alloy-steel plates for pressure vessels, high-strength-steel plates for marine structures or industrial machinery, and the like include high-quality extra-heavy steel plates that have thicknesses of more than 100 mm and that are to be used as important members. High-quality extra-heavy steel plates may have a problem in the internal quality thereof in terms of use performance. Therefore, in the related art, large-sized ingots are manufactured by an ingot casting method, and the large-sized ingots are rolled or forged at a sufficient reduction ratio to thereby manufacture high-quality extra-heavy steel plates. A manufacturing method that improves the internal quality of high-quality extra-heavy steel plates is thus performed.

Meanwhile, since productivity in the ingot casting method is low, a method in which extra-thick slabs having large slab thicknesses are manufactured by vertical continuous casting has been attempted. One example of the method is described in Patent Literature 1. It is disclosed that, in the method described in Patent Literature 1, when the thickness of a slab is 380 mm or more, the casting speed is set to 0.2 m/min or less due to limitation of the machine length of continuous casting machine or to prevent bulging deformation of the slab.

When an extra-thick slab (hereinafter referred to as the slab) is produced using a vertical-bending type continuous casting machine, a stress is applied to the slab in a bending section, in which the slab that has been withdrawn in a direction substantially parallel to the vertical direction from a mold is bent in a direction substantially parallel to the horizontal direction. Therefore, a risk of corner cracks/transverse cracks occurring in the slab increases. Patent Literature 2 describes one example of a continuous casting machine that reduces such a risk. In the vertical-bending type continuous casting machine described in Patent Literature 2, manufacturing conditions suitable for the chemical components and the thickness of a slab to be manufactured are set so that a slab without surface defects and without internal cracks is manufactured. Specifically, the chemical components of the slab described in Patent Literature 2 are C: 0.05 to 0.55 mass%, Si: 0.10 to 2.00 mass%, Mn: 0.30 to 1.90 mass%, P: 0.005 to 0.070 mass%, and S: 0.003 to 0.120 mass%. The thickness of the slab is 280 to 350 mm. The slab is cast by the vertical-bending type continuous casting machine in which a casting speed is set to 0.7 to 1.1 m/min and a specific water flow rate is set to 0.15 to 0.40 l/kg·steel. In addition, in that case, a vertical length, a bending length, a secondary cooling length, an arc length, a straightening length, and the like are each set within a previously set range.

### Citation List

### Patent Literature

Patent Literature 1: Japanese Unexamined Patent Application Publication No. 2007-229736
Patent Literature 2: Japanese Unexamined Patent Application Publication No. 2009-274116

### Summary of Invention

### Technical Problem

In the method described in Patent Literature 1, the casting speed is limited to 0.2 m/min or lower when the thickness of the slab is 380 mm or more. That is, when the thickness of the slab is 380 mm or more, productivity of the slab in the method described in Patent Literature 1 is low, and there is still room for improvement in this respect.

In the vertical-bending type continuous casting machine described in Patent Literature 2, the thickness of the slab with which both productivity and suppression of surface cracks can be addressed is 280 to 350 mm. Therefore, when the thickness of the slab is 350 mm or more, addressing both productivity and suppression of surface cracks may not be possible, and there is still room for improvement in this respect.

The present invention has been made to solve the aforementioned problems, and an object of the present invention is to provide a slab continuous-casting method capable of improving productivity of a slab that has a thickness larger than that of conventional slab and capable of ensuring surface quality of the slab by suppressing surface cracks of the slab.

### Solution to Problem

Means for solving the aforementioned problems are as follows.
[1] A slab continuous-casting method using a continuous casting machine that includes a mold, a vertical section disposed downstream of the mold in a moving direction of a slab withdrawn from a mold, a bending section disposed downstream of the vertical section in the moving direction, and a horizontal section disposed downstream of the bending section in the moving direction, in which a surface temperature of the slab at an exit side of the vertical section is 700°C or higher and 1200°C or lower, and in which a first cooling density X calculated from an amount of cooling water in the bending section is less than or equal to a second cooling density Y calculated from an amount of cooling water in the horizontal section.
[2] The slab continuous-casting method according to [1], in which cooling water is to be supplied to the slab in each of the vertical section, the bending section, and the horizontal section, in which the first cooling density X is a value obtained by dividing a total supply amount of cooling water to be supplied to the slab inside the bending section by a surface area of the slab inside the bending section, and in which the second cooling density Y is a value obtained by dividing a total supply amount of cooling water to be supplied to the slab inside the horizontal section by a surface area of the slab inside the horizontal section.
[3] The slab continuous-casting method according to [1] or [2], in which a thickness of the slab is 350 mm or more and 500 mm or less.
[4] The slab continuous-casting method according any one of [1] to [3], in which a withdrawal speed of the slab in the vertical section is 0.2 to 1.5 m/min.

### Advantageous Effects of Invention

According to the present invention, an extra-thick slab that has favorable internal quality with fewer surface cracks or without surface cracks and that has a larger slab thickness than that of conventional slab can be continuously cast at a higher speed than that in conventional method. Therefore, it is possible to improve productivity of a slab that has a thickness larger than that of conventional slab. Brief Description of Drawings

[Fig. 1] Fig. 1 illustrates one example of a vertical-bending type continuous casting machine to which the slab continuous-casting method according to the present embodiment is applicable.

### Description of Embodiments

Hereinafter, the present invention will be specifically described through an embodiment (hereinafter referred to as the present embodiment) of the present invention. The present embodiment described below is one suitable example of the present invention, and the present invention should not be limited by this example in any way.

A slab continuous-casting method according to the present embodiment is a method in which an extra-thick slab that has favorable internal quality with fewer surface cracks or without surface cracks and that has a thickness larger than that of conventional slab is continuously cast at a higher speed than that in conventional method by optimizing the amount of cooling in a secondary cooling zone of a continuous casting machine. Fig. 1 illustrates one example of a continuous casting machine to which the slab continuous-casting method according to the present embodiment is applicable. The continuous casting machine 1 illustrated in Fig. 1 is of a so-called vertical bending type, and, in the continuous casting machine 1, an immersion nozzle 4 is attached to a bottom portion of a tundish 2 via a sliding nozzle 3. Molten steel 5 is supplied to the tundish 2 from a ladle, which is not illustrated. The sliding nozzle 3 is a device that regulates the amount of the molten steel 5 that is to be supplied from the tundish 2 to a mold 6 through the immersion nozzle 4.

A cooling channel, which is not illustrated, is formed in the mold 6, and cooling water is supplied to the cooling channel from a cooling-water supply source, which is not illustrated. In the mold 6, heat is removed from the molten steel 5 into the cooling water to thereby form a slab 7 having a surface on which a solidified shell is formed, and the slab 7 is withdrawn from the mold 6 in a direction substantially parallel to the vertical direction. Therefore, an unsolidified layer in which the molten steel 5 has not yet solidified is formed inside the slab 7 directly below the mold. Note that the mold 6 may be referred to as the primary cooling zone. In Fig. 1, the unsolidified layer is hatched.

In the present embodiment, the thickness of the slab 7 that is to be withdrawn from the mold 6 of the continuous casting machine 1 illustrated in Fig. 1 is set to 350 to 500 mm. In addition, the withdrawal speed of the slab 7 from the mold 6 is set to 0.2 to 1.5 m/min. The withdrawal speed is a withdrawal speed in a steady state. Note that the steady state means a state in which a pouring speed during a period from which a period of starting pouring, a period of terminating pouring, a period of slab connection, and the like are excluded is constant. When the withdrawal speed of the slab 7 is less than 0.2 m/min, the molten steel 5 may be solidified inside the mold 6 and may disable the withdrawal of the slab 7 from the mold 6. When the withdrawal speed of the slab 7 is higher than 1.5 m/min, there is a possibility that the solidified shell is not sufficiently formed and causes a break-out in which the molten steel leaks due to the solidified shell being broken when the slab 7 is withdrawn from the mold 6. Therefore, the withdrawal speed of the slab 7 is preferably set to 0.2 to 1.5 m/min. The withdrawal speed of the slab 7 is more preferably set to 0.3 to 1.4 m/min.

A secondary cooling zone is provided below the mold 6 of the continuous casting machine 1. Specifically, a vertical section 8 extending in a direction substantially parallel to the vertical direction to support the slab 7 that is continuously withdrawn from the mold 6 is provided directly below the mold 6. The vertical section 8 includes a plurality of slab support rolls 9. As illustrated in Fig. 1, these slab support rolls 9 are disposed on two sides of the slab 7 in the thickness direction of the slab 7 and are disposed to be spaced from each other in a direction substantially parallel to the vertical direction. The slab support rolls 9 support the slab 7 that has been withdrawn from the mold 6. Therefore, the space between the slab support rolls 9 in the thickness direction of the slab 7 is set to be substantially the same as the thickness of the slab 7 immediately after being withdrawn from the mold 6. In addition, cooling water is to be supplied into the slab support rolls 9. Note that each slab support roll 9 of the vertical section 8, each slab support roll 9 of a bending section 10, which is described later, and each slab support roll 9 of a horizontal section 11, which is described later, are configured to be substantially the same. An example of each slab support roll 9 thereof is a roll that is manufactured by overlay-welding 13Cr4Ni onto a surface of a base material containing 21CrMoV511.

The bending section 10 is provided downstream of the vertical section 8 in the moving direction of the slab 7. The bending section 10 is configured to cause the slab 7 that has been withdrawn from the mold 6 in a direction substantially parallel to the vertical direction to be bent in a direction substantially parallel to the horizontal direction. The bending section 10 includes a plurality of segments. As illustrated in Fig. 1, the segments are arranged in an arc shape such that the vertical section 8 and the horizontal section 11 are smoothly connected. Each of the segments includes a plurality of the slab support rolls 9. These slab support rolls 9 are disposed on two sides of the slab 7 in the thickness direction of the slab 7 and are disposed to be spaced from each other along the above-described arc shape, in other words, in the moving direction of the slab 7. The space between the slab support rolls 9 of the bending section 10 in the thickness direction of the slab 7 is set to be substantially the same as the thickness of the slab 7 that is immediately after being withdrawn from the mold 6. Note that, in Fig. 1, a first segment 10a, a second segment 10b, and a final segment 10c are illustrated while illustration of other segments is omitted for simplification of the drawings. The first segment 10a is located at the most upstream position in the moving direction of the slab 7 among the plurality of segments of the bending section 10. The second segment 10b is located downstream of the first segment 10a. The final segment 10c is located at the most downstream position in the moving direction of the slab.

The first segment 10a and the vertical section 8 are adjacent to each other. In the first segment 10a, the slab 7 that has exited the vertical section 8 and that has a flat shape is to be bent. The final segment 10c and the horizontal section 11 are adjacent to each other. In the final segment 10c, the slab 7 that is curved is to be shaped into its original flat shape. Note that, in the following description, the first segment 10a is referred to as the upper shaping zone 10a, and the final segment 10c is referred to as the lower shaping zone 10c.

The horizontal section 11 extends in a direction substantially parallel to the horizontal direction. In addition, similarly to the bending section 10, the horizontal section 11 includes a plurality of segments. In the example illustrated in Fig. 1, the horizontal section 11 is constituted by two segments. Each of the segments includes a plurality of the slab support rolls 9. These slab support rolls 9 are disposed on two sides of the slab 7 in the thickness direction of the slab 7 and are disposed to be spaced from each other in a direction substantially parallel to the horizontal direction. The space between the slab support rolls 9 of the horizontal section 11 in the thickness direction of the slab 7 is set such that a target thickness of the slab is achieved at the exit side of the continuous casting machine 1.

In addition, in each of the vertical section 8, the bending section 10, and the horizontal section 11, a spray nozzle, which is not illustrated, is disposed between each pair of the slab support rolls 9 adjacent to each other in the moving direction of the slab 7. The slab 7 is to be cooled by cooling water that is sprayed from these spray nozzles onto the slab 7. The vertical section 8, the bending section 10, the horizontal section 11, and each spray nozzle, which are provided below the mold 6 as described above, correspond to the above-described secondary cooling zone. Although details are not illustrated, the distance between a leading end portion of each spray nozzle and the slab 7 in the thickness direction of the slab 7 is set to approximately 90 mm. In addition, the temperature of the cooling water ejected from each spray nozzle onto the slab 7 may be approximately 15°C or higher and 45°C or lower in one example.

A slab cutting machine 12 that cuts the slab 7 is provided downstream of the horizontal section 11 in the moving direction of the slab 7. The slab 7 that has completed its solidification in the horizontal section 11 is cut to a predetermined length by the slab cutting machine 12.

In addition, the continuous casting machine 1 illustrated in Fig. 1 is configured such that the supply amount of the cooling water to be supplied to each of the vertical section 8, the bending section 10, and the horizontal section 11 can be controlled independently. Specifically, a cooling-water supply source 14 is connected to each of the spray nozzles of the vertical section 8, each of the spray nozzles of the bending section 10, and each of the spray nozzles of the horizontal section 11 via respective flow-rate controllers 13. The control of the supply amount of the cooling water by the flow-rate controllers 13 may be performed by a control device, which is not illustrated, or by an operator. In addition, the flow-rate controllers 13 may be, for example, flow-rate control valves.

In the present embodiment, each of cooling densities X and Y of the cooling water in the bending section 10 and the horizontal section 11 is set to avoid formation of surface cracks in the slab 7 due to bending or shaping of the slab 7 in the upper shaping zone 10a or the lower shaping zone 10c. In other words, when the surface temperature of the slab 7 in the upper shaping zone 10a and the lower shaping zone 10c is within a brittle temperature range of the slab 7, surface cracks of the slab 7 may be formed due to bending or shaping of the slab 7. Therefore, a cooling density ratio X/Y between the first cooling density X in the bending section 10 and the second cooling density Y in the horizontal section 11 is set to 1.0 or less so as to cause the slab 7 to pass, with a temperature higher than the brittle temperature range of the slab 7, through the upper shaping zone 10a and the lower shaping zone 10c. In other words, the first cooling density X is set to be less than or equal to the second cooling density Y.

The first cooling density X is a value that is obtained by dividing the total supply amount (hereinafter simply referred to as total amount) of the cooling water that is to be supplied to the slab 7 inside the bending section 10 by the surface area of the slab 7 inside the bending section 10. The second cooling density Y is a value that is obtained by dividing the total amount of the cooling water that is supplied to the slab 7 inside the horizontal section 11 by the surface area of the slab 7 inside the horizontal section 11.

The surface area of the slab 7 inside the bending section 10 and the surface area of the slab 7 inside the horizontal section 11 can be obtained on the basis of design. The total amount of the cooling water in the bending section 10 means the total amount of the cooling water that is supplied to the slab 7 in the bending section 10 when the slab 7 is continuously cast using one charge of the molten steel 5. Similarly to this, the total amount of the cooling water in the horizontal section 11 means the total amount of the cooling water that is supplied to the slab 7 in the horizontal section 11 when continuous casting using one charge of the molten steel 5 is performed. In addition, one charge means the molten steel 5 in the same lot. The brittle temperature range means a temperature range in which surface cracks are easily formed due to bending or shaping of the slab 7.

When the cooling density ratio X/Y is more than 1.0, an amount of cooling water in the horizontal section 11 and the second cooling density Y calculated on the basis of the amount of the cooling water are less than an amount of cooling water in the bending section 10 and the first cooling density X calculated on the basis of the amount of the cooling water, respectively. Therefore, cooling of the slab 7 in the horizontal section 11 may be insufficient and may result in incomplete solidification of the slab 7. In addition, the surface temperature of the slab 7 may enter the brittle temperature range when the slab 7 passes through the upper shaping zone 10a or the lower shaping zone 10c in the bending section 10 and may cause surface cracks in the slab 7. Meanwhile, when the cooling density ratio X/Y is 0.0 and when, for example, the first cooling density X in the bending section 10 is 0.0, that is, when an amount of cooling water in the bending section 10 is 0.0, the solidified shell of the slab 7 directly below the mold 6 becomes excessively thinner than in the above-described steady state. Consequently, large bulging may occur, and withdrawal of the slab 7 from the mold 6 may become impossible. Therefore, the cooling density ratio X/Y is preferably greater than 0.0 and less than or equal to 1.0 and is more preferably greater than 0.0 and less than or equal to 0.9.

### (Operations and Effects)

Operations and effects of the present embodiment will be described. The slab 7 having a thickness of 350 to 500 mm is withdrawn from the mold 6. The withdrawal speed of the slab 7 is set to 0.2 to 1.5 m/min. In the vertical section 8, cooling water is sprayed from spray nozzles onto the slab 7. The surface temperature is thus decreased to a previously set temperature. In the present embodiment, the surface temperature of the slab 7 at the exit side of the vertical section 8 is preferably 700 to 1200°C. For example, when the surface temperature of the slab 7 at the exit side of the vertical section 8 is less than 700°C, the surface temperature of the slab 7 enters the brittle temperature range when the slab 7 passes through the upper shaping zone 10a or the lower shaping zone 10c, and may cause surface cracks in the slab 7. Meanwhile, when the surface temperature of the slab 7 at the exit side of the vertical section 8 is higher than 1200°C, a withdrawal failure may occur due to increasing bulging.

Next, the slab 7 is curved in the upper shaping zone 10a of the bending section 10, and the slab 7 is moved in this state toward the horizontal section 11. Also in the bending section 10, the cooling water is sprayed from each spray nozzle onto the slab 7. In the present embodiment, as described above, the cooling density ratio X/Y between the first cooling density X inside the bending section 10 and the second cooling density Y inside the horizontal section 11 is set to 1.0 or less. In other words, the first cooling density X for the slab 7 inside the bending section 10 is set to be less than the second cooling density Y for the slab inside the horizontal section 11. Therefore, cooling of the slab 7 in the bending section 10 is suppressed compared with cooling in the horizontal section 11. Consequently, the surface temperature of the slab 7 is maintained at a temperature higher than the brittle temperature range, and, in this state, the slab 7 reaches the lower shaping zone 10c. Then, the slab 7 is shaped in the lower shaping zone 10c from a curved shape into an original flat shape. Next, the cooling water is sprayed onto the slab 7 from each spray nozzle also in the horizontal section 11, and the slab 7 is completely solidified throughout the inside thereof.

As described above, according to the present embodiment, the surface temperature of the slab 7 in each of the shaping zones 10a and 10c is maintained at a temperature higher than the brittle temperature range. Therefore, according to the present embodiment, the extra-thick slab 7 that has favorable internal quality with fewer surface cracks or without surface cracks and that has a thickness larger than that of conventional slab can be continuously cast at a higher speed than that in conventional method. Therefore, it is possible to improve productivity of the extra-thick slab 7 that has a thickness larger than that of conventional slab.

Note that the present invention is not limited to the above-described embodiment. For example, a control device, which is not illustrated, that controls the continuous casting machine 1 illustrated in Fig. 1 may be included, and cooling of the slab 7 in the secondary cooling zone may be controlled by the control device. In other words, the amount of the cooling water that is to be sprayed in the vertical section 8 from each spray nozzle onto the slab 7 is controlled by the above-described control device. The surface temperature of the slab 7 at the exit side of the vertical section 8 is thereby set to 700 to 1200°C. In addition, the amount of the cooling water that is to be sprayed in each of the bending section 10 and the horizontal section 11 from each spray nozzle onto the slab 7 is controlled by the control device. The cooling density ratio X/Y is thereby controlled to be 1.0 or less. Even in such a configuration, the same operations and effects as those in the above-described embodiment can be obtained.

In addition, although the slab 7 is cooled by the cooling water sprayed in the secondary cooling zone onto the slab 7 in the present embodiment described above, dry casting in which cooling water is not sprayed onto the slab 7 may be employed instead. Note that, in the dry casting, sprays disposed directly below the mold 6 are operated to prevent failures in withdrawal of the slab **7.** However, sprays of the bending section 10 are not operated. Meanwhile, sprays of the horizontal section 11 are operated. As a result, the cooling density ratio X/Y in the dry casting has a value substantially equal to zero.

### EXAMPLES

Next, examples conducted to confirm effects of the slab continuous-casting method according to the present embodiment will be described. In the examples, slabs of various grades for each of which test conditions were changed were continuously cast using a continuous casting machine configured to be the same as that in the above-described embodiment. Specifically, slabs each having a thickness: 350 to 450 mm were continuously cast at a casting speed: 0.4 to 1.2 m/mim with molten steel for normal steel having carbon content: 0.07 to 0.50 mass%. Then, the occurrence status of surface cracks in each of the continuously cast slabs was evaluated. Table 1 lists chemical compositions of each steel grade used in the examples. Table 2 lists the steel grades of the slabs continuously cast in the examples, the pouring speed, that is, the withdrawal speed of each slab, the slab thicknesses, and the secondary cooling conditions. Note that the water flow density in Table 2 corresponds to the cooling density in the present embodiment.

**[Table 1]**

| Steel Grade | Chemical Compositions (mass%, balance Fe, and impurities) | | | | | |
|---|---|---|---|---|---|---|
| | C | Si | Mn | P | S | Sol.Al |
| a | 0.07 | 0.34 | 1.52 | 0.05 | 0.002 | 0.035 |
| b | 0.16 | 0.33 | 1.50 | 0.15 | 0.003 | 0.027 |
| c | 0.50 | 0.18 | 0.65 | 0.10 | 0.004 | 0.023 |

**[Table 2]**

| Test No. | Steel Grade | Withdrawal Speed | Slab Thickness | Secondary Cooling Conditions | | | Crack Occurrence Status |
|---|---|---|---|---|---|---|---|
| | | | | X: Water Flow Density in Curved Section | Y: Water Flow Density in Horizontal Section | X/Y | |
| | | (m/min) | (mm) | (L/m²) | (L/m²⁾ | | |
| 1 | c | 0.5 | 450 | 17 | 7 | 2.43 | occurred |
| 2 | b | 0.7 | 400 | 25 | 11 | 2.27 | occurred |
| 3 | a | 1 | 350 | 35 | 17 | 2.06 | occurred |
| 4 | c | 0.9 | 400 | 31 | 11 | 2.82 | occurred |
| 5 | b | 1.2 | 350 | 55 | 30 | 1.83 | occurred |
| 6 | c | 0.5 | 450 | 32 | 43 | 0.74 | favorable |
| 7 | b | 0.6 | 400 | 23 | 52 | 0.44 | favorable |
| 8 | c | 1 | 350 | 17 | 65 | 0.26 | favorable |
| 9 | b | 0.6 | 400 | 21 | 37 | 0.57 | favorable |
| 10 | a | 0.4 | 500 | 12 | 48 | 0.25 | favorable |

### (Method of Checking Surface Cracks)

A method of checking surface cracks will be described. Both surfaces of each slab manufactured under the conditions shown in Table 2 were each cut off by approximately 2 mm. Thereafter, surface cracks in each surface of the slab after cutting were detected through penetrant testing (also referred to as color check). Then, the number of surface cracks in each surface of the slab was counted, and, when the total number of surface cracks in the slab was three or less, the slab was evaluated as "favorable", which means that surface cracks were suppressed compared with conventional slab. In addition, when the total number of surface cracks was more than three, the slab was evaluated as "occurred", which means that surface cracks were substantially the same as those in conventional slab. Table 2 lists these evaluation results together with the above-described manufacturing conditions. The test numbers 1 to 5 listed in Table 2 are comparative examples for which various manufacturing conditions are out of the range specified in the present invention. The test numbers 6 to 10 are examples for which various manufacturing conditions are within the range specified in the present invention.

### (Evaluation)

As shown in Table 2, the slabs manufactured under the conditions of the test numbers 1 to 5, which were comparative examples, were evaluated as "occurred". The slabs manufactured under the conditions of the test numbers 6 to 10, which were examples, were evaluated as "favorable". Accordingly, it was confirmed that carrying out the slab continuous-casting method according to the present invention in the manufacture of a slab having a thickness larger than that of conventional slab at a higher speed than that in conventional method can prevent or suppress occurrence of surface cracks in the slab.

### Reference Signs List

- 1: continuous casting machine
- 2: tundish
- 3: sliding nozzle
- 4: immersion nozzle
- 5: molten steel
- 6: mold
- 7: slab
- 8: vertical section
- 9: slab support roll
- 10: bending section
- 10a: first segment, upper shaping zone
- 10b: second segment
- 10c: final segment, lower shaping zone
- 11: horizontal section
- 12: slab cutting machine
- 13: flow-rate controller
- 14: cooling-water supply source

## Claims

1. A slab continuous-casting method using a continuous casting machine that includes a mold, a vertical section disposed downstream of the mold in a moving direction of a slab withdrawn from a mold, a bending section disposed downstream of the vertical section in the moving direction, and a horizontal section disposed downstream of the bending section in the moving direction,
wherein a surface temperature of the slab at an exit side of the vertical section is 700°C or higher and 1200°C or lower, and
wherein a first cooling density X calculated from an amount of cooling water in the bending section is less than or equal to a second cooling density Y calculated from an amount of cooling water in the horizontal section.

2. The slab continuous-casting method according to claim 1,
wherein cooling water is to be supplied to the slab in each of the vertical section, the bending section, and the horizontal section,
wherein the first cooling density X is a value obtained by dividing a total supply amount of cooling water to be supplied to the slab inside the bending section by a surface area of the slab inside the bending section, and
wherein the second cooling density Y is a value obtained by dividing a total supply amount of cooling water to be supplied to the slab inside the horizontal section by a surface area of the slab inside the horizontal section.

3. The slab continuous-casting method according to claim 1 or 2, wherein a thickness of the slab is 350 mm or more and 500 mm or less.

4. The slab continuous-casting method according to claim 1 or 2, wherein a withdrawal speed of the slab in the vertical section is 0.2 to 1.5 m/min.

5. The slab continuous-casting method according to claim 3, wherein a withdrawal speed of the slab in the vertical section is 0.2 to 1.5 m/min.
